



US009034058B2

(12) **United States Patent**  
**Robinson et al.**

(10) **Patent No.:** **US 9,034,058 B2**  
(45) **Date of Patent:** **\*May 19, 2015**

- (54) **AGGLOMERATED PARTICULATE LOW-RANK COAL FEEDSTOCK AND USES THEREOF**
- (71) Applicant: **GreatPoint Energy, Inc.**, Cambridge, MA (US)
- (72) Inventors: **Earl T. Robinson**, Lakeland, FL (US); **Kenneth P. Keckler**, Naperville, IL (US); **Pattabhi K. Raman**, Kildeer, IL (US); **Avinash Sirdeshpande**, Chicago, IL (US)
- (73) Assignee: **GreatPoint Energy, Inc.**, Cambridge, MA (US)
- (\*) Notice: Subject to any disclaimer, the term of this patent is extended or adjusted under 35 U.S.C. 154(b) by 0 days.  
This patent is subject to a terminal disclaimer.
- (21) Appl. No.: **14/039,454**
- (22) Filed: **Sep. 27, 2013**

(65) **Prior Publication Data**

US 2014/0091259 A1 Apr. 3, 2014

- Related U.S. Application Data**
- (60) Provisional application No. 61/708,104, filed on Oct. 1, 2012, provisional application No. 61/775,775, filed on Mar. 11, 2013.
- (51) **Int. Cl.**  
*C01B 31/14* (2006.01)  
*C10J 3/46* (2006.01)  
*C10L 5/10* (2006.01)  
*C10L 5/36* (2006.01)
- (52) **U.S. Cl.**  
CPC .... *C10J 3/46* (2013.01); *C10L 5/10* (2013.01); *C10L 5/363* (2013.01)
- (58) **Field of Classification Search**  
USPC ..... 23/314, 313 R  
See application file for complete search history.

(56) **References Cited**

## U.S. PATENT DOCUMENTS

- 2,605,215 A 7/1952 Coghlan  
2,694,623 A 11/1954 Welty, Jr. et al.  
2,791,549 A 5/1957 Jahnig  
2,813,126 A 11/1957 Tierney  
2,860,959 A 11/1958 Pettyjohn et al.  
2,866,405 A 5/1959 Benson et al.  
3,034,848 A 5/1962 King  
3,114,930 A 12/1963 Oldham et al.  
3,150,716 A 9/1964 Strelzoff et al.  
3,164,330 A 1/1965 Neidl  
3,351,563 A 11/1967 Negra et al.  
3,435,590 A 4/1969 Smith  
3,531,917 A 10/1970 Grunewald et al.  
3,544,291 A 12/1970 Schlinger et al.  
3,594,985 A 7/1971 Ameen et al.

- 3,615,300 A 10/1971 Holm et al.  
3,689,240 A 9/1972 Aldridge et al.  
3,740,193 A 6/1973 Aldridge et al.  
3,746,522 A 7/1973 Donath  
3,759,036 A 9/1973 White  
3,779,725 A 12/1973 Hegarty et al.  
3,814,725 A 6/1974 Zimmerman et al.  
3,817,725 A 6/1974 Sieg et al.  
3,828,474 A 8/1974 Quartulli  
3,833,327 A 9/1974 Pitzer et al.  
3,847,567 A 11/1974 Kalina et al.  
3,876,393 A 4/1975 Kasai et al.  
3,904,386 A 9/1975 Graboski et al.  
3,915,670 A 10/1975 Lacey et al.  
3,920,229 A 11/1975 Piggott  
3,929,431 A 12/1975 Koh et al.  
3,958,957 A 5/1976 Koh et al.  
3,966,875 A 6/1976 Bratzler et al.  
3,969,089 A 7/1976 Moss et al.  
3,971,639 A 7/1976 Matthews  
3,972,693 A 8/1976 Wiesner et al.  
3,975,168 A 8/1976 Gorbaty  
3,985,519 A 10/1976 Kalina et al.  
3,989,811 A 11/1976 Hill  
3,996,014 A 12/1976 Muller et al.  
3,998,607 A 12/1976 Wesslhoft et al.  
3,999,607 A 12/1976 Pennington et al.  
4,005,996 A 2/1977 Hausberger et al.  
4,011,066 A 3/1977 Bratzler et al.  
4,017,272 A 4/1977 Anwer et al.  
4,021,370 A 5/1977 Harris et al.

(Continued)

## FOREIGN PATENT DOCUMENTS

- CA 966660 4/1975  
CA 1003217 1/1977

(Continued)  
OTHER PUBLICATIONS

- U.S. Appl. No. 12/778,538, filed May 12, 2010, Robinson, et al.  
U.S. Appl. No. 12/778,548, filed May 12, 2010, Robinson, et al.  
U.S. Appl. No. 12/778,552, filed May 12, 2010, Robinson, et al.  
Asami, K., et al., "Highly Active Iron Catalysts from Ferric Chloride or the Steam Gasification of Brown Coal," *ind. Eng. Chem. Res.*, vol. 32, No. 8, 1993, pp. 1631-1636.  
Berger, R. et al., "High Temperature CO<sub>2</sub>-Absorption: A Process Offering New Prospects in Fuel Chemistry," *The Fifth International Symposium on Coal Combustion*, Nov. 2003, Nanjing, China, pp. 547-549.  
Brown et al., "Biomass-Derived Hydrogen From a Thermally Basted Gasifier," Aug. 2005.  
Brown et al., "Biomass-Derived Hydrogen From a Thermally Basted Gasifier," *DOE Hydrogen Program Contractors' Review Meeting*, Center for Sustainable Environmental Technologies, Iowa State University, May 21, 2003.

(Continued)

*Primary Examiner* — Edward Johnson(74) *Attorney, Agent, or Firm* — McDonnell Boehnen Hulbert & Berghoff LLP(57) **ABSTRACT**

The present invention relates generally to processes for preparing agglomerated particulate low-rank coal feedstocks of a particle size suitable for reaction in certain gasification reactors and, in particular, for coal gasification. The present invention also relates to integrated coal gasification processes including preparing and utilizing such agglomerated particulate low-rank coal feedstocks.

| (56)                  | References Cited |                                         |
|-----------------------|------------------|-----------------------------------------|
| U.S. PATENT DOCUMENTS |                  |                                         |
| 4,025,423 A           | 5/1977           | Stonner et al.                          |
| 4,044,098 A           | 8/1977           | Miller et al.                           |
| 4,046,523 A           | 9/1977           | Kalina et al.                           |
| 4,052,176 A           | 10/1977          | Child et al.                            |
| 4,053,554 A           | 10/1977          | Reed et al.                             |
| 4,057,512 A           | 11/1977          | Vadovic et al.                          |
| 4,069,304 A           | 1/1978           | Starkovich et al.                       |
| 4,077,778 A           | 3/1978           | Nahas et al.                            |
| 4,091,073 A           | 5/1978           | Winkler                                 |
| 4,092,125 A           | 5/1978           | Stambaugh et al.                        |
| 4,094,650 A           | 6/1978           | Koh et al.                              |
| 4,100,256 A           | 7/1978           | Bozzelli et al.                         |
| 4,101,449 A           | 7/1978           | Noda et al.                             |
| 4,104,201 A           | 8/1978           | Banks et al.                            |
| 4,113,615 A           | 9/1978           | Gorbaty                                 |
| 4,116,996 A           | 9/1978           | Huang                                   |
| 4,118,204 A           | 10/1978          | Eakman et al.                           |
| 4,152,119 A           | 5/1979           | Schulz                                  |
| 4,157,246 A           | 6/1979           | Eakman et al.                           |
| 4,159,195 A           | 6/1979           | Clavenna                                |
| 4,162,902 A           | 7/1979           | Wiesner et al.                          |
| 4,173,465 A           | 11/1979          | Meissner et al.                         |
| 4,189,307 A           | 2/1980           | Marion                                  |
| 4,193,771 A           | 3/1980           | Sharp et al.                            |
| 4,193,772 A           | 3/1980           | Sharp                                   |
| 4,200,439 A           | 4/1980           | Lang                                    |
| 4,204,843 A           | 5/1980           | Neavel                                  |
| 4,211,538 A           | 7/1980           | Eakman et al.                           |
| 4,211,669 A           | 7/1980           | Eakman et al.                           |
| 4,219,338 A           | 8/1980           | Wolfs et al.                            |
| 4,223,728 A           | 9/1980           | Pegg                                    |
| 4,225,457 A           | 9/1980           | Schulz                                  |
| 4,235,044 A           | 11/1980          | Cheung                                  |
| 4,243,639 A           | 1/1981           | Haas et al.                             |
| 4,249,471 A           | 2/1981           | Gunnerman                               |
| 4,252,771 A           | 2/1981           | Lagana et al.                           |
| 4,260,421 A           | 4/1981           | Brown et al.                            |
| 4,265,868 A           | 5/1981           | Kamody                                  |
| 4,270,937 A           | 6/1981           | Adler et al.                            |
| 4,284,416 A           | 8/1981           | Nahas                                   |
| 4,292,048 A           | 9/1981           | Wesselhoft et al.                       |
| 4,298,584 A           | 11/1981          | Makrides                                |
| 4,315,753 A           | 2/1982           | Bruckensteine et al.                    |
| 4,315,758 A           | 2/1982           | Patel et al.                            |
| 4,318,712 A           | 3/1982           | Lang et al.                             |
| 4,322,222 A           | 3/1982           | Sass                                    |
| 4,330,305 A           | 5/1982           | Kuessner et al.                         |
| 4,331,451 A           | 5/1982           | Isogaya et al.                          |
| 4,334,893 A           | 6/1982           | Lang                                    |
| 4,336,034 A           | 6/1982           | Lang et al.                             |
| 4,336,233 A           | 6/1982           | Appl et al.                             |
| 4,341,531 A           | 7/1982           | Duranleau et al.                        |
| 4,344,486 A           | 8/1982           | Parrish                                 |
| 4,347,063 A           | 8/1982           | Sherwood et al.                         |
| 4,348,486 A           | 9/1982           | Calvin et al.                           |
| 4,348,487 A           | 9/1982           | Calvin et al.                           |
| 4,353,713 A           | 10/1982          | Cheng                                   |
| 4,365,975 A           | 12/1982          | Williams et al.                         |
| 4,372,755 A           | 2/1983           | Tolman et al.                           |
| 4,375,362 A           | 3/1983           | Moss                                    |
| 4,385,905 A           | 5/1983           | Tucker                                  |
| 4,397,656 A           | 8/1983           | Ketkar                                  |
| 4,400,182 A           | 8/1983           | Davies et al.                           |
| 4,407,206 A           | 10/1983          | Bartok et al.                           |
| 4,428,535 A           | 1/1984           | Venetucci                               |
| 4,432,773 A           | 2/1984           | Euker, Jr. et al.                       |
| 4,433,065 A           | 2/1984           | Van Der Burgt et al.                    |
| 4,436,028 A           | 3/1984           | Wilder                                  |
| 4,436,531 A           | 3/1984           | Estabrook et al.                        |
| 4,439,210 A           | 3/1984           | Lancet                                  |
| 4,443,415 A           | 4/1984           | Queneau et al.                          |
| 4,444,568 A           | 4/1984           | Beisswenger et al.                      |
| 4,459,138 A           | 7/1984           | Soung                                   |
| 4,462,814 A           | 7/1984           | Holmes et al.                           |
| 4,466,828 A           | 8/1984           | Tamai et al.                            |
|                       |                  | 4,468,231 A 8/1984 Bartok et al.        |
|                       |                  | 4,478,425 A 10/1984 Benko               |
|                       |                  | 4,478,725 A 10/1984 Velling et al.      |
|                       |                  | 4,482,529 A 11/1984 Chen et al.         |
|                       |                  | 4,491,609 A 1/1985 Degel et al.         |
|                       |                  | 4,497,784 A 2/1985 Diaz                 |
|                       |                  | 4,500,323 A 2/1985 Siegfried et al.     |
|                       |                  | 4,505,881 A 3/1985 Diaz                 |
|                       |                  | 4,508,544 A 4/1985 Moss                 |
|                       |                  | 4,508,693 A 4/1985 Diaz                 |
|                       |                  | 4,515,604 A 5/1985 Eisenlohr et al.     |
|                       |                  | 4,515,764 A 5/1985 Diaz                 |
|                       |                  | 4,524,050 A 6/1985 Chen et al.          |
|                       |                  | 4,540,681 A 9/1985 Kustes et al.        |
|                       |                  | 4,541,841 A 9/1985 Reinhardt            |
|                       |                  | 4,551,155 A 11/1985 Wood et al.         |
|                       |                  | 4,558,027 A 12/1985 McKee et al.        |
|                       |                  | 4,572,826 A 2/1986 Moore                |
|                       |                  | 4,594,140 A 6/1986 Cheng                |
|                       |                  | 4,597,775 A 7/1986 Billimoria et al.    |
|                       |                  | 4,597,776 A 7/1986 Ullman et al.        |
|                       |                  | 4,604,105 A 8/1986 Aquino et al.        |
|                       |                  | 4,609,388 A 9/1986 Adler et al.         |
|                       |                  | 4,609,456 A 9/1986 Deschamps et al.     |
|                       |                  | 4,617,027 A 10/1986 Lang                |
|                       |                  | 4,619,864 A 10/1986 Hendrix et al.      |
|                       |                  | 4,620,421 A 11/1986 Brown et al.        |
|                       |                  | 4,661,237 A 4/1987 Kimura et al.        |
|                       |                  | 4,668,428 A 5/1987 Najjar               |
|                       |                  | 4,668,429 A 5/1987 Najjar               |
|                       |                  | 4,675,035 A 6/1987 Appfel               |
|                       |                  | 4,678,480 A 7/1987 Heinrich et al.      |
|                       |                  | 4,682,986 A 7/1987 Lee et al.           |
|                       |                  | 4,690,814 A 9/1987 Velenyi et al.       |
|                       |                  | 4,696,678 A 9/1987 Koyama et al.        |
|                       |                  | 4,699,632 A 10/1987 Babu et al.         |
|                       |                  | 4,704,136 A 11/1987 Weston et al.       |
|                       |                  | 4,720,289 A 1/1988 Vaugh et al.         |
|                       |                  | 4,747,938 A 5/1988 Khan                 |
|                       |                  | 4,781,731 A 11/1988 Schlinger           |
|                       |                  | 4,803,061 A 2/1989 Najjar et al.        |
|                       |                  | 4,808,194 A 2/1989 Najjar et al.        |
|                       |                  | 4,810,475 A 3/1989 Chu et al.           |
|                       |                  | 4,822,935 A 4/1989 Scott                |
|                       |                  | 4,848,983 A 7/1989 Tomita et al.        |
|                       |                  | 4,854,944 A 8/1989 Strong               |
|                       |                  | 4,861,346 A 8/1989 Najjar et al.        |
|                       |                  | 4,861,360 A 8/1989 Appfel               |
|                       |                  | 4,872,886 A 10/1989 Henley et al.       |
|                       |                  | 4,876,080 A 10/1989 Paulson             |
|                       |                  | 4,892,567 A 1/1990 Yan                  |
|                       |                  | 4,960,450 A 10/1990 Schwarz et al.      |
|                       |                  | 4,995,193 A 2/1991 Soga et al.          |
|                       |                  | 5,017,282 A 5/1991 Delbianco et al.     |
|                       |                  | 5,055,181 A 10/1991 Maa et al.          |
|                       |                  | 5,057,294 A 10/1991 Sheth et al.        |
|                       |                  | 5,059,406 A 10/1991 Sheth et al.        |
|                       |                  | 5,074,357 A 12/1991 Haines              |
|                       |                  | 5,093,094 A 3/1992 Van Kleeck et al.    |
|                       |                  | 5,094,737 A 3/1992 Bearden, Jr. et al.  |
|                       |                  | 5,132,007 A 7/1992 Meyer et al.         |
|                       |                  | 5,223,173 A 6/1993 Jeffrey              |
|                       |                  | 5,225,044 A 7/1993 Breu                 |
|                       |                  | 5,236,557 A 8/1993 Muller et al.        |
|                       |                  | 5,242,470 A 9/1993 Salter et al.        |
|                       |                  | 5,250,083 A 10/1993 Wolfenbarger et al. |
|                       |                  | 5,277,884 A 1/1994 Shinnar et al.       |
|                       |                  | 5,388,645 A 2/1995 Puri et al.          |
|                       |                  | 5,388,650 A 2/1995 Michael              |
|                       |                  | 5,435,940 A 7/1995 Doering et al.       |
|                       |                  | 5,536,893 A 7/1996 Gudmundsson          |
|                       |                  | 5,566,755 A 10/1996 Seidle et al.       |
|                       |                  | 5,616,154 A 4/1997 Elliott et al.       |
|                       |                  | 5,630,854 A 5/1997 Sealock, Jr. et al.  |
|                       |                  | 5,641,327 A 6/1997 Leas                 |
|                       |                  | 5,660,807 A 8/1997 Forg et al.          |
|                       |                  | 5,669,960 A 9/1997 Couche               |
|                       |                  | 5,670,122 A 9/1997 Zamansky et al.      |
|                       |                  | 5,720,785 A 2/1998 Baker                |

| (56)                  | References Cited |                          |
|-----------------------|------------------|--------------------------|
| U.S. PATENT DOCUMENTS |                  |                          |
| 5,733,515 A           | 3/1998           | Doughty et al.           |
| 5,769,165 A           | 6/1998           | Bross et al.             |
| 5,776,212 A           | 7/1998           | Leas                     |
| 5,788,724 A           | 8/1998           | Carugati et al.          |
| 5,855,631 A           | 1/1999           | Leas                     |
| 5,865,898 A           | 2/1999           | Holtzapple et al.        |
| 5,968,465 A           | 10/1999          | Koveal et al.            |
| 6,013,158 A           | 1/2000           | Wootton                  |
| 6,015,104 A           | 1/2000           | Rich, Jr.                |
| 6,028,234 A           | 2/2000           | Heinemann et al.         |
| 6,032,737 A           | 3/2000           | Brady et al.             |
| 6,090,356 A           | 7/2000           | Jahnke et al.            |
| 6,119,778 A           | 9/2000           | Seidle et al.            |
| 6,132,478 A           | 10/2000          | Tsurui et al.            |
| 6,180,843 B1          | 1/2001           | Heinemann et al.         |
| 6,187,465 B1          | 2/2001           | Galloway                 |
| 6,379,645 B1          | 4/2002           | Bucci et al.             |
| 6,389,820 B1          | 5/2002           | Rogers et al.            |
| 6,419,888 B1          | 7/2002           | Wyckoff                  |
| 6,506,349 B1          | 1/2003           | Khanmamedov              |
| 6,506,361 B1          | 1/2003           | Machado et al.           |
| 6,602,326 B2          | 8/2003           | Lee et al.               |
| 6,641,625 B1          | 11/2003          | Clawson et al.           |
| 6,653,516 B1          | 11/2003          | Yoshikawa et al.         |
| 6,692,711 B1          | 2/2004           | Alexion et al.           |
| 6,790,430 B1          | 9/2004           | Lackner et al.           |
| 6,797,253 B2          | 9/2004           | Lyon                     |
| 6,808,543 B2          | 10/2004          | Paisley                  |
| 6,830,597 B1          | 12/2004          | Green                    |
| 6,855,852 B1          | 2/2005           | Jackson et al.           |
| 6,878,358 B2          | 4/2005           | Vosteen et al.           |
| 6,894,183 B2          | 5/2005           | Choudhary et al.         |
| 6,955,595 B2          | 10/2005          | Kim                      |
| 6,955,695 B2          | 10/2005          | Nahas                    |
| 6,969,494 B2          | 11/2005          | Herbst                   |
| 7,056,359 B1          | 6/2006           | Somerville et al.        |
| 7,074,373 B1          | 7/2006           | Warren et al.            |
| 7,077,202 B2          | 7/2006           | Shaw et al.              |
| 7,100,692 B2          | 9/2006           | Parsley et al.           |
| 7,118,720 B1          | 10/2006          | Mendelsohn et al.        |
| 7,132,183 B2          | 11/2006          | Galloway                 |
| 7,168,488 B2          | 1/2007           | Olsvik et al.            |
| 7,205,448 B2          | 4/2007           | Gajda et al.             |
| 7,220,502 B2          | 5/2007           | Galloway                 |
| 7,299,868 B2          | 11/2007          | Zapadinski               |
| 7,309,383 B2          | 12/2007          | Beech, Jr. et al.        |
| 7,481,275 B2          | 1/2009           | Olsvik et al.            |
| 7,666,383 B2          | 2/2010           | Green                    |
| 7,677,309 B2          | 3/2010           | Shaw et al.              |
| 7,758,663 B2          | 7/2010           | Rabovitser et al.        |
| 7,897,126 B2          | 3/2011           | Rappas et al.            |
| 7,901,644 B2          | 3/2011           | Rappas et al.            |
| 7,922,782 B2          | 4/2011           | Sheth                    |
| 7,926,750 B2          | 4/2011           | Hauserman                |
| 7,976,593 B2          | 7/2011           | Graham                   |
| 8,114,176 B2          | 2/2012           | Nahas                    |
| 8,114,177 B2          | 2/2012           | Hippo et al.             |
| 8,123,827 B2          | 2/2012           | Robinson                 |
| 8,163,048 B2          | 4/2012           | Rappas et al.            |
| 8,192,716 B2          | 6/2012           | Raman et al.             |
| 8,202,913 B2          | 6/2012           | Robinson et al.          |
| 8,268,899 B2          | 9/2012           | Robinson et al.          |
| 8,286,901 B2          | 10/2012          | Rappas et al.            |
| 8,297,542 B2          | 10/2012          | Rappas et al.            |
| 8,328,890 B2          | 12/2012          | Reiling et al.           |
| 8,349,037 B2          | 1/2013           | Steiner et al.           |
| 8,349,039 B2          | 1/2013           | Robinson                 |
| 8,361,428 B2          | 1/2013           | Raman et al.             |
| 8,366,795 B2          | 2/2013           | Raman et al.             |
| 8,479,833 B2          | 7/2013           | Raman                    |
| 8,479,834 B2          | 7/2013           | Preston                  |
| 8,502,007 B2          | 8/2013           | Hippo et al.             |
| 2002/0036086 A1       | 3/2002           | Minkkinen et al.         |
| 2003/0070808 A1       | 4/2003           | Allison                  |
| 2003/0131582 A1       | 7/2003           | Anderson et al.          |
|                       | 2003/0167691 A1  | 9/2003 Nahas             |
|                       | 2004/0020123 A1  | 2/2004 Kimura et al.     |
|                       | 2004/0023086 A1  | 2/2004 Su et al.         |
|                       | 2004/0123601 A1  | 7/2004 Fan               |
|                       | 2004/0180971 A1  | 9/2004 Inoue et al.      |
|                       | 2004/0256116 A1  | 12/2004 Olsvik et al.    |
|                       | 2005/0107648 A1  | 5/2005 Kimura et al.     |
|                       | 2005/0137442 A1  | 6/2005 Gajda et al.      |
|                       | 2005/0192362 A1  | 9/2005 Rodriguez et al.  |
|                       | 2005/0287056 A1  | 12/2005 Baker et al.     |
|                       | 2005/0288537 A1  | 12/2005 Maund et al.     |
|                       | 2006/0149423 A1  | 7/2006 Barnicki et al.   |
|                       | 2006/0228290 A1  | 10/2006 Green            |
|                       | 2006/0231252 A1  | 10/2006 Shaw et al.      |
|                       | 2006/0265953 A1  | 11/2006 Hobbs            |
|                       | 2006/0272813 A1  | 12/2006 Olsvik et al.    |
|                       | 2007/0000177 A1  | 1/2007 Hippo et al.      |
|                       | 2007/0051043 A1  | 3/2007 Schingnitz        |
|                       | 2007/0083072 A1  | 4/2007 Nahas             |
|                       | 2007/0180990 A1  | 8/2007 Downs et al.      |
|                       | 2007/0186472 A1  | 8/2007 Rabovister et al. |
|                       | 2007/0220810 A1  | 9/2007 Leveson et al.    |
|                       | 2007/0227729 A1  | 10/2007 Zubrin et al.    |
|                       | 2007/0237696 A1  | 10/2007 Payton           |
|                       | 2007/0277437 A1  | 12/2007 Sheth            |
|                       | 2007/0280218 A1  | 12/2007 Jenkins          |
|                       | 2008/0022586 A1  | 1/2008 Gilbert et al.    |
|                       | 2008/0141591 A1  | 6/2008 Kohl              |
|                       | 2008/0289822 A1  | 11/2008 Betzer Tsilevich |
|                       | 2009/0012188 A1  | 1/2009 Rojey et al.      |
|                       | 2009/0048476 A1  | 2/2009 Rappas et al.     |
|                       | 2009/0090055 A1  | 4/2009 Ohtsuka           |
|                       | 2009/0090056 A1  | 4/2009 Ohtsuka           |
|                       | 2009/0165361 A1  | 7/2009 Rappas et al.     |
|                       | 2009/0165376 A1  | 7/2009 Lau et al.        |
|                       | 2009/0165379 A1  | 7/2009 Rappas            |
|                       | 2009/0165380 A1  | 7/2009 Lau et al.        |
|                       | 2009/0165381 A1  | 7/2009 Robinson          |
|                       | 2009/0165382 A1  | 7/2009 Rappas et al.     |
|                       | 2009/0165383 A1  | 7/2009 Rappas et al.     |
|                       | 2009/0165384 A1  | 7/2009 Lau et al.        |
|                       | 2009/0166588 A1  | 7/2009 Spitz et al.      |
|                       | 2009/0169448 A1  | 7/2009 Rappas et al.     |
|                       | 2009/0169449 A1  | 7/2009 Rappas et al.     |
|                       | 2009/0170968 A1  | 7/2009 Nahas et al.      |
|                       | 2009/0173079 A1  | 7/2009 Wallace et al.    |
|                       | 2009/0217575 A1  | 9/2009 Raman et al.      |
|                       | 2009/0217582 A1  | 9/2009 May et al.        |
|                       | 2009/0217584 A1  | 9/2009 Raman et al.      |
|                       | 2009/0217585 A1  | 9/2009 Raman et al.      |
|                       | 2009/0217586 A1  | 9/2009 Rappas et al.     |
|                       | 2009/0217587 A1  | 9/2009 Raman et al.      |
|                       | 2009/0217588 A1  | 9/2009 Hippo et al.      |
|                       | 2009/0217589 A1  | 9/2009 Robinson          |
|                       | 2009/0217590 A1  | 9/2009 Rappas et al.     |
|                       | 2009/0218424 A1  | 9/2009 Hauserman         |
|                       | 2009/0220406 A1  | 9/2009 Rahman            |
|                       | 2009/0229182 A1  | 9/2009 Raman et al.      |
|                       | 2009/0235585 A1  | 9/2009 Neels et al.      |
|                       | 2009/0236093 A1  | 9/2009 Zubrin et al.     |
|                       | 2009/0246120 A1  | 10/2009 Raman et al.     |
|                       | 2009/0259080 A1  | 10/2009 Raman et al.     |
|                       | 2009/0260287 A1  | 10/2009 Lau              |
|                       | 2009/0305093 A1  | 12/2009 Biollaz et al.   |
|                       | 2009/0324458 A1  | 12/2009 Robinson et al.  |
|                       | 2009/0324459 A1  | 12/2009 Robinson et al.  |
|                       | 2009/0324460 A1  | 12/2009 Robinson et al.  |
|                       | 2009/0324461 A1  | 12/2009 Robinson et al.  |
|                       | 2009/0324462 A1  | 12/2009 Robinson et al.  |
|                       | 2010/0018113 A1  | 1/2010 Bohlig et al.     |
|                       | 2010/0050654 A1  | 3/2010 Chiu et al.       |
|                       | 2010/0071235 A1  | 3/2010 Pan et al.        |
|                       | 2010/0071262 A1  | 3/2010 Robinson et al.   |
|                       | 2010/0076235 A1  | 3/2010 Reiling et al.    |
|                       | 2010/0120926 A1  | 5/2010 Robinson et al.   |
|                       | 2010/0121125 A1  | 5/2010 Hippo et al.      |
|                       | 2010/0159352 A1  | 6/2010 Gelin et al.      |
|                       | 2010/0168494 A1  | 7/2010 Rappas et al.     |
|                       | 2010/0168495 A1  | 7/2010 Rappas et al.     |

| (56)                     | References Cited |                     |    |             |         |  |
|--------------------------|------------------|---------------------|----|-------------|---------|--|
| U.S. PATENT DOCUMENTS    |                  |                     |    |             |         |  |
| 2010/0179232 A1          | 7/2010           | Robinson et al.     | GB | 996327      | 6/1965  |  |
| 2010/0287835 A1          | 11/2010          | Reiling et al.      | GB | 1033764     | 6/1966  |  |
| 2010/0287836 A1          | 11/2010          | Robinson et al.     | GB | 1448562     | 9/1976  |  |
| 2010/0292350 A1          | 11/2010          | Robinson et al.     | GB | 1453081     | 10/1976 |  |
| 2011/0031439 A1          | 2/2011           | Sirdeshpande et al. | GB | 1467219     | 3/1977  |  |
| 2011/0062012 A1          | 3/2011           | Robinson            | GB | 1467995     | 3/1977  |  |
| 2011/0062721 A1          | 3/2011           | Sirdeshpande et al. | GB | 1599 932    | 7/1977  |  |
| 2011/0062722 A1          | 3/2011           | Sirdeshpande et al. | GB | 1560873     | 2/1980  |  |
| 2011/0064648 A1          | 3/2011           | Preston et al.      | GB | 2078251     | 1/1982  |  |
| 2011/0088896 A1          | 4/2011           | Preston             | GB | 2154600     | 9/1985  |  |
| 2011/0088897 A1          | 4/2011           | Raman               | GB | 2455864     | 6/2009  |  |
| 2011/0146978 A1          | 6/2011           | Perlman             | JP | 53-94305    | 8/1978  |  |
| 2011/0146979 A1          | 6/2011           | Wallace             | JP | 53-111302   | 9/1978  |  |
| 2011/0197501 A1          | 8/2011           | Taulbee             | JP | 54020003    | 2/1979  |  |
| 2011/0207002 A1          | 8/2011           | Powell et al.       | JP | 54-150402   | 11/1979 |  |
| 2011/0217602 A1          | 9/2011           | Sirdeshpande        | JP | 55-12181    | 1/1980  |  |
| 2011/0262323 A1          | 10/2011          | Rappas et al.       | JP | 56-145982   | 11/1981 |  |
| 2011/0294905 A1          | 12/2011          | Robinson et al.     | JP | 56157493    | 12/1981 |  |
| 2012/0046510 A1          | 2/2012           | Sirdeshpande        | JP | 60-35092    | 2/1985  |  |
| 2012/0060417 A1          | 3/2012           | Raman et al.        | JP | 60-77938    | 5/1985  |  |
| 2012/0102836 A1          | 5/2012           | Raman et al.        | JP | 62241991    | 10/1987 |  |
| 2012/0102837 A1          | 5/2012           | Raman et al.        | JP | 62 257985   | 11/1987 |  |
| 2012/0210635 A1          | 8/2012           | Edwards             | JP | 03-115491   | 5/1991  |  |
| 2012/0213680 A1          | 8/2012           | Rappas et al.       | JP | 2000290659  | 10/2000 |  |
| 2012/0271072 A1          | 10/2012          | Robinson et al.     | JP | 2000290670  | 10/2000 |  |
| 2012/0305848 A1          | 12/2012          | Sirdeshpande        | JP | 2002105467  | 4/2002  |  |
| 2013/0042824 A1          | 2/2013           | Sirdeshpande        | JP | 2004292200  | 10/2004 |  |
| 2013/0046124 A1          | 2/2013           | Sirdeshpande        | JP | 2004298818  | 10/2004 |  |
| 2013/0172640 A1          | 7/2013           | Robinson et al.     | JP | 2006 169476 | 6/2006  |  |
| FOREIGN PATENT DOCUMENTS |                  |                     |    |             |         |  |
| CA 1041553               | 10/1978          |                     | WO | 00/18681    | 4/2000  |  |
| CA 1106178               | 8/1981           |                     | WO | 00/43468    | 7/2000  |  |
| CA 1 125 026             | 6/1982           |                     | WO | 02/40768    | 5/2002  |  |
| CA 1187702               | 6/1985           |                     | WO | 02/079355   | 10/2002 |  |
| CA 1282243               | 4/1991           |                     | WO | 02/103157   | 12/2002 |  |
| CA 1299589               | 4/1992           |                     | WO | 03/018958   | 3/2003  |  |
| CA 1332108               | 9/1994           |                     | WO | 03/033624   | 4/2003  |  |
| CA 2673121               | 6/2008           |                     | WO | 2004/055323 | 7/2004  |  |
| CA 2713642               | 7/2009           |                     | WO | 2004/072210 | 8/2004  |  |
| CN 1477090               | 2/2004           |                     | WO | 2006/031011 | 3/2006  |  |
| CN 101555420             | 10/2009          |                     | WO | 2007/005284 | 1/2007  |  |
| DE 2 210 891             | 3/1972           |                     | WO | 2007/047210 | 4/2007  |  |
| DE 2210891               | 9/1972           |                     | WO | 2007/068682 | 6/2007  |  |
| DE 2852710               | 6/1980           |                     | WO | 2007/076363 | 7/2007  |  |
| DE 3422202               | 12/1985          |                     | WO | 2007/077137 | 7/2007  |  |
| DE 100610607             | 6/2002           |                     | WO | 2007/077138 | 7/2007  |  |
| EP 0024792               | 3/1981           |                     | WO | 2007/083072 | 7/2007  |  |
| EP 0 067 580             | 12/1982          |                     | WO | 2007/128370 | 11/2007 |  |
| EP 102828                | 3/1984           |                     | WO | 2007/143376 | 12/2007 |  |
| EP 0 138 463             | 4/1985           |                     | WO | 2008/058636 | 5/2008  |  |
| EP 0 225 146             | 6/1987           |                     | WO | 2008/073889 | 6/2008  |  |
| EP 0 259 927             | 3/1988           |                     | WO | 2008/087154 | 7/2008  |  |
| EP 0473153               | 3/1992           |                     | WO | 2009/018053 | 2/2009  |  |
| EP 0 723 930             | 7/1996           |                     | WO | 2009/048723 | 4/2009  |  |
| EP 819                   | 4/2000           |                     | WO | 2009/048724 | 4/2009  |  |
| EP 1001002               | 5/2000           |                     | WO | 2009/086361 | 7/2009  |  |
| EP 1004746               | 5/2000           |                     | WO | 2009/086362 | 7/2009  |  |
| EP 1136542               | 9/2001           |                     | WO | 2009/086363 | 7/2009  |  |
| EP 1 207 132             | 5/2002           |                     | WO | 2009/086366 | 7/2009  |  |
| EP 1 741 673             | 6/2006           |                     | WO | 2009/086367 | 7/2009  |  |
| EP 1768207               | 3/2007           |                     | WO | 2009/086370 | 7/2009  |  |
| EP 2058471               | 5/2009           |                     | WO | 2009/086372 | 7/2009  |  |
| FR 797 089               | 4/1936           |                     | WO | 2009/086374 | 7/2009  |  |
| FR 2 478 615             | 9/1981           |                     | WO | 2009/086377 | 7/2009  |  |
| FR 2906879               | 4/2008           |                     | WO | 2009/086383 | 7/2009  |  |
| GB 593910                | 10/1947          |                     | WO | 2009/086407 | 7/2009  |  |
| GB 640907                | 8/1950           |                     | WO | 2009/086408 | 7/2009  |  |
| GB 676615                | 7/1952           |                     | WO | 2009/111330 | 9/2009  |  |
| GB 701 131               | 12/1953          |                     | WO | 2009/111331 | 9/2009  |  |
| GB 760627                | 11/1956          |                     | WO | 2009/111332 | 9/2009  |  |
| GB 798741                | 7/1958           |                     | WO | 2009/111335 | 9/2009  |  |
| GB 820 257               | 9/1959           |                     | WO | 2009/111342 | 9/2009  |  |
|                          |                  |                     | WO | 2009/111345 | 9/2009  |  |
|                          |                  |                     | WO | 2009/124017 | 10/2009 |  |
|                          |                  |                     | WO | 2009/124019 | 10/2009 |  |
|                          |                  |                     | WO | 2009/158576 | 12/2009 |  |
|                          |                  |                     | WO | 2009/158579 | 12/2009 |  |
|                          |                  |                     | WO | 2009/158580 | 12/2009 |  |
|                          |                  |                     | WO | 2009/158582 | 12/2009 |  |
|                          |                  |                     | WO | 2009/158583 | 12/2009 |  |

(56)

## References Cited

## FOREIGN PATENT DOCUMENTS

WO 2010/033846 3/2010  
 WO 2010/033848 3/2010  
 WO 2010/033850 3/2010  
 WO 2010/033852 3/2010  
 WO 2010/048493 4/2010  
 WO 2010/078297 7/2010  
 WO 2010/078298 7/2010  
 WO 2010/132549 11/2010  
 WO 2010/132551 11/2010  
 WO 2011/017630 2/2011  
 WO 2011/029278 3/2011  
 WO 2011/029282 3/2011  
 WO 2011/029283 3/2011  
 WO 2011/029284 3/2011  
 WO 2011/029285 3/2011  
 WO 2011/034888 3/2011  
 WO 2011/034889 3/2011  
 WO 2011/034890 3/2011  
 WO 2011/034891 3/2011  
 WO 2011/049858 4/2011  
 WO 2011/049861 4/2011  
 WO 2011/063608 6/2011  
 WO 2011/084580 7/2011  
 WO 2011/084581 7/2011  
 WO 2011/106285 9/2011  
 WO 2011/139694 11/2011  
 WO 2011/150217 12/2011  
 WO 2012/024369 2/2012  
 WO 2012/033997 3/2012  
 WO 2012/061235 5/2012  
 WO 2012/061238 5/2012  
 WO 2012/116003 8/2012  
 WO 2012/145497 10/2012  
 WO 2012/166879 12/2012  
 WO 2013/025808 2/2013  
 WO 2013/025812 2/2013  
 WO 2013/052553 4/2013

## OTHER PUBLICATIONS

Cohen, S.J., Project Manager, "Large Pilot Plant Alternatives for Scaleup of the Catalytic Coal Gasification Process," FE-2480-20, U.S. Dept. of Energy, Contract No. EX-76-C-01-2480, 1979.  
 Euker, Jr., C.A., Reitz, R.A., Program Managers, "Exxon Catalytic Coal-Gasification-Process Development Program," Exxon Research & Engineering Company, FE-2777-31, U.S. Dept. of Energy, Contract No. ET-78-C-01-2777, 1981.  
 Kalina, T., Nahas, N.C., Project Managers, "Exxon Catalytic Coal Gasification Process Predevelopment Program," Exxon Research & Engineering Company, FE-2369-24, U.S. Dept. of Energy, Contract No. E(49-18)-2369, 1978.  
 Nahas, N.C., "Exxon Catalytic Coal Gasification Process—Fundamentals to Flowsheets," Fuel, vol. 62, No. 2, 1983, pp. 239-241.  
 Ohtsuka, Y. et al., "Highly Active Catalysts from Inexpensive Raw Materials for Coal Gasification," Catalysis Today, vol. 39, 1997, pp. 111-125.  
 Ohtsuka, Yasuo et al., "Steam Gasification of Low-Rank Coals with a Chlorine-Free Iron Catalyst from Ferric Chloride," Ind. Eng. Chem. Res., vol. 30, No. 8, 1991, pp. 1921-1926.  
 Ohtsuka, Yasuo et al., "Calcium Catalysed Steam Gasification of Yalourn Brown Coal," Fuel, vol. 65, 1986, pp. 1653-1657.  
 Ohtsuka, Yasuo, et al., "Iron-Catalyzed Gasification of Brown Coal at Low Temperatures," Energy & Fuels, vol. 1, No. 1, 1987, pp. 32-36.  
 Ohtsuka, Yasuo, et al., "Ion-Exchanged Calcium From Calcium Carbonate and Low-Rank Coals: High Catalytic Activity in Steam Gasification," Energy & Fuels 1996, 10, pp. 431-435.  
 Ohtsuka, Yasuo et al., "Steam Gasification of Coals with Calcium Hydroxide," Energy & Fuels, vol. 9, No. 6, 1995, pp. 1038-1042.  
 Pereira, P. et al., "Catalytic Steam Gasification of Coals," Energy & Fuels, vol. 6, No. 4, 1992, pp. 407-410.  
 Ruan Xiang-Quan, et al., "Effects of Catalysis on Gasification of Tatong Coal Char," Fuel, vol. 66, Apr. 1987, pp. 568-571.  
 Tandon, D., "Low Temperature and Elevated Pressure Steam Gasification of Illinois Coal," College of Engineering in the Graduate School, Southern Illinois University at Carbondale, Jun. 1996.  
 Adsorption, <http://en.wikipedia.org/wiki/Adsorption>, pp. 1-8, (Oct. 17, 2007).  
 Amine gas treating, [http://en.wikipedia.org/wiki/Acid\\_gas\\_removal](http://en.wikipedia.org/wiki/Acid_gas_removal), pp. 1-4 (Oct. 21, 2007).  
 Coal, [http://en.wikipedia.org/wiki/Coal\\_gasification](http://en.wikipedia.org/wiki/Coal_gasification), pp. 1-8 (Oct. 29, 2007).  
 Coal Data: A Reference, Energy Information Administration, Office of Coal, Nuclear, Electric, and Alternate Fuels U.S. Department of Energy, DOE/EIA-0064(93), Feb. 1995.  
 Deepak Tandon, Dissertation Approval, "Low Temperature and Elevated Pressure Steam Gasification of Illinois Coal", Jun. 13, 1996.  
 Demibras, "Deminerization of Agricultural Residues by Water Leaching", *Energy Sources*, vol. 25, pp. 679-687, (2003).  
 Fluidized Bed Gasifiers, [http://www.energypproducts.com/fluidized\\_bed\\_gasifiers.htm](http://www.energypproducts.com/fluidized_bed_gasifiers.htm) Oct. 2007, pp. 1-5.  
 Gas separation, [http://en.wikipedia.org/wiki/Gas\\_separation](http://en.wikipedia.org/wiki/Gas_separation), pp. 1-2 (Feb. 24, 2007).  
 Gasification, <http://en.wikipedia.org/wiki/Gasification>, pp. 1-6 (Oct. 29, 2007).  
 Gallagher Jr., et al., "Catalytic Coal Gasification for SNG Manufacture", *Energy Research*, vol. 4, pp. 137-147, (1980).  
 Heinemann, et al., "Fundamental and Exploratory Studies of Catalytic Steam Gasification of Carbonaceous Materials", Final Report Fiscal Years 1985-1994.  
 Jensen, et al. Removal of K and C1 by leaching of straw char, *Biomass and Bioenergy*, vol. 20, pp. 447-457, (2001).  
 Mengjie, et al., "A potential renewable energy resource development and utilization of biomass energy", <http://www.fao.org/docrep/T4470E/t4470e0n.htm>, pp. 1-8 (1994).  
 Meyers, et al. Fly Ash as a Construction Material for Highways, A Manual. Federal Highway Administration, Report No. FHWA-IP-76-16, Washington, DC, 1976.  
 Moulton, Lyle K. "Bottom Ash and Boiler Slag", *Proceedings of the Third International Ash Utilization Symposium*, U.S. Bureau of Mines, Information Circular No. 8640, Washington, DC, 1973.  
 Natural gas processing, [http://en.wikipedia.org/wiki/Natural\\_gas\\_processing](http://en.wikipedia.org/wiki/Natural_gas_processing), pp. 1-4 (Oct. 22, 2007).  
 Natural Gas Processing: The Crucial Link Between Natural Gas Production and Its Transportation to Market. Energy Information Administration, Office of Oil and Gas; pp. 1-11, (2006).  
 Prins, et al., "Exergetic optimisation of a production process of Fischer-Tropsch fuels from biomass", *Fuel Processing Technology*, vol. 86, pp. 375-389, (2004).  
 Reboiler, <http://en.wikipedia.org/wiki/Reboiler>, pp. 1-4 (Nov. 11, 2007).  
 What is XPS?, <http://www.nuance.northwestern.edu/KeckII/xps1.asp>, 2006, pp. 1-2 (2006).  
 2.3 Types of gasifiers, <http://www.fao.org/docrep/t0512e/T0512e0a.htm>, pp. 1-6 (1986).  
 2.4 Gasification fuels, <http://www.fao.org/docrep/t0512e/T0512e0b.htm#TopOfPage>, pp. 1-8 (1986).  
 2.5 Design of downdraught gasifiers, <http://www.fao.org/docrep/t0512e/T0512e0c.htm#TopOfPage>, pp. 1-8 (1986).  
 2.6 Gas cleaning and cooling, <http://www.fao.org/docrep/t0512e0d.htm#TopOfPage>, pp. 1-3 (1986).  
 A.G. Collot et al., "Co-pyrolysis and co-gasification of coal and biomass in bench-scale fixed-bed and fluidized bed reactors", (1999) Fuel 78, pp. 667-679.  
 Wenkui Zhu et al., "Catalytic gasification of char from co-pyrolysis of coal and biomass", (2008) Fuel Processing Technology, vol. 89, pp. 890-896.  
 Chiesa P. et al., "Co-Production of hydrogen, electricity and CO2 from coal with commercially ready technology. Part A: Performance and emissions", (2005) International Journal of Hydrogen Energy, vol. 30, No. 7, pp. 747-767.  
 Chiaramonte et al., "Upgrade Coke by Gasification", (1982) Hydrocarbon Processing, vol. 61 (9), pp. 255-257 (Abstract only).  
 Gerdes, Kristin, et al., "Integrated Gasification Fuel Cell Performance and Cost Assessment," National Energy Technology Laboratory, U.S. Department of Energy, Mar. 27, 2009, pp. 1-26.

(56)

**References Cited**

## OTHER PUBLICATIONS

- Ghosh, S., et al., "Energy Analysis of a Cogeneration Plant Using Coal Gasification and Solid Oxide Fuel Cell," *Energy*, 2006, vol. 31, No. 2-3, pp. 345-363.
- Jeon, S.K., et al., "Characteristics of Steam Hydrogasification of Wood Using a Micro-Batch Reactor," *Fuel*, 2007, vol. 86, pp. 2817-2823.
- Li, Mu, et al., "Design of Highly Efficient Coal-Based Integrated Gasification Fuel Cell Power Plants," *Journal of Power Sources*, 2010, vol. 195, pp. 5707-5718.

Prins, M.J., et al., "Exergetic Optimisation of a Production Process of Fischer-Tropsch Fuels from Biomass," *Fuel Processing Technology*, 2005, vol. 86, No. 4, pp. 375-389.

Hydromethanation Process, GreatPoint Energy, Inc., from World Wide Web <<http://greatpointenergy.com/ourtechnology.php>> accessed Sep. 5, 2013.

Sigma-Aldrich "Particle Size Conversion Table" (2004); from World Wide Web <<http://www.sigmaaldrich.com/chemistry/learning-center/technical-library/particle-size-conversion.printview.html>>.



FIGURE 1



FIGURE 2

**AGGLOMERATED PARTICULATE  
LOW-RANK COAL FEEDSTOCK AND USES  
THEREOF**

**CROSS-REFERENCE TO RELATED  
APPLICATIONS**

This application claims priority under 35 U.S.C. §119 from U.S. Provisional Application Ser. Nos. 61/708,104 (filed 1 Oct. 2012) and 61/775,775 (filed 11 Mar. 2013), the disclosures of which are incorporated by reference herein for all purposes as if fully set forth.

This application is related to U.S. application Ser. No. 14/039,321, entitled AGGLOMERATED PARTICULATE LOW-RANK COAL FEEDSTOCK AND USES THEREOF, U.S. application Ser. No. 14/039,402, entitled AGGLOMERATED PARTICULATE LOW-RANK COAL FEEDSTOCK AND USES THEREOF, and U.S. application Ser. No. 14/040,058, entitled USE OF CONTAMINATED LOW-RANK COAL FOR COMBUSTION, all of which are concurrently filed herewith and incorporated by reference herein for all purposes as if fully set forth.

**FIELD OF THE INVENTION**

The present invention relates generally to processes for preparing agglomerated particulate low-rank coal feedstocks of a particle size suitable for reaction in certain gasification reactors and, in particular, for coal gasification. The present invention also relates to an integrated coal gasification process including preparing and utilizing such agglomerated particulate low-rank coal feedstocks.

**BACKGROUND OF THE INVENTION**

In view of numerous factors such as higher energy prices and environmental concerns, the production of value-added products (such as pipeline-quality substitute natural gas, hydrogen, methanol, higher hydrocarbons, ammonia and electrical power) from lower-fuel-value carbonaceous feedstocks (such as petroleum coke, resids, asphaltenes, coal and biomass) is receiving renewed attention.

Such lower-fuel-value carbonaceous feedstocks can be gasified at elevated temperatures and pressures to produce a synthesis gas stream that can subsequently be converted to such value-added products.

Certain gasification processes, such as those based on partial combustion/oxidation and/or steam gasification of a carbon source at elevated temperatures and pressures (thermal gasification), generate syngas (carbon monoxide+hydrogen, lower BTU synthesis gas stream) as the primary product (little or no methane is directly produced). The syngas can be directly combusted for heat energy, and/or can be further processed to produce methane (via catalytic methanation, see reaction (III) below), hydrogen (via water-gas shift, see reaction (II) below) and/or any number of other higher hydrocarbon products.

Such lower-fuel-value carbonaceous feedstocks can alternatively be directly combusted for their heat value, typically for generating steam and electrical energy (directly or indirectly via generated steam).

In the above uses, the raw particulate feedstocks are typically processed by at least grinding to a specified particle size profile (including upper and lower end as well as  $dp(50)$  of a particle size distribution) suitable for the particular gasification operation. Typically particle size profiles will depend on the type of bed, fluidization conditions (in the case of fluidized beds, such as fluidizing medium and velocity) and other

conditions such as feedstock composition and reactivity, feedstock physical properties (such as density and surface area), reactor pressure and temperature, reactor configuration (such as geometry and internals), and a variety of other factors generally recognized by those of ordinary skill in the relevant art.

“Low-rank” coals are typically softer, friable materials with a dull, earthy appearance. They are characterized by relatively higher moisture levels and relatively lower carbon content, and therefore a lower energy content. Examples of low-rank coals include peat, lignite and sub-bituminous coals. Examples of “high-rank” coals include bituminous and anthracite coals.

In addition to their relatively low heating values, the use of low-ranks coals has other drawbacks. For example, the friability of such coals can lead to high fines losses in the feedstock preparation (grinding and other processing) and in the gasification/combustion of such coals. Such fines must be managed or even disposed of, which usually means an economic and efficiency hit (economic and processing disincentive) to the use of such coals. For very highly friable coals such as lignite, such fines losses can approach or even exceed 50% of the original material. In other words, the processing and use of low-rank coals can result in a loss (or less desired use) of a material percentage of the carbon content in the low-rank coal as mined.

It would, therefore, be desirable to find a way to efficiently process low-rank coals to reduce fines losses in both the feedstock processing and ultimate conversion of such low-rank coal materials in various gasification and combustion processes.

Low-rank coals that contain significant amounts of impurities, such as sodium and chlorine (e.g., NaCl), may actually be unusable in gasification processes due to the highly corrosive and fouling nature of such components, thus requiring pretreatment to remove such impurities. Typically the addition of such a pretreatment renders the use of sodium and/or chlorine contaminated low-rank coals economically unfeasible.

It would, therefore, be desirable to find a way to more efficiently pretreat these contaminated low-rank coals to removed a substantial portion of at least the inorganic sodium and/or chlorine content.

Low-rank coals may also have elevated ash levels, and thus lower useable carbon content per unit raw feedstock.

It would, therefore, be desirable to find a way to more efficiently pretreat these low-rank coals to reduce overall ash content.

Also, low-ranks coals tend to have lower bulk density and more variability in individual particle density than high-rank coals, which can create challenges for designing and operating gasification and combustion processes.

It would, therefore, be desirable to find a way to increase both particle density and particle density consistency of low-rank coals, to ultimately improve the operability of processes that utilize such low-rank coals.

**SUMMARY OF THE INVENTION**

In a first aspect, the invention provides a process for preparing a free-flowing agglomerated particulate low-rank coal feedstock of a specified particle size distribution, the process comprising the steps of:

(a) selecting a specification for the particle size distribution of the free-flowing agglomerated particulate low-rank coal feedstock, the specification comprising

- (i) a target upper end particle size of about 72600 microns of less;
- (ii) a target lower end particle size of about 6350 microns or greater, and
- (iii) a target  $dp(50)$  between the target upper end particle size and target lower end particle size;
- (b) providing a raw particulate low-rank coal feedstock having an initial particle density;
- (c) grinding the raw particulate low-rank coal feedstock to a ground  $dp(50)$  of from about 2% to about 50% of the target  $dp(50)$ , to generate a ground low-rank coal feedstock;
- (d) pelletizing the ground low-rank coal feedstock with water and a binder to generate free-flowing agglomerated low-rank coal particles having a pelletized  $dp(50)$  of from about 90% to about 110% of the target  $dp(50)$ , and a particle density of at least about 5% greater than the initial particle density, wherein the binder is selected from the group consisting of a water-soluble binder, a water-dispersible binder and a mixture thereof; and
- (e) removing about 90 wt % or greater of
  - (i) particles larger than the upper end particle size, and
  - (ii) particles smaller than the lower end particle size,
 from the free-flowing agglomerated low-rank coal particles to generate the free-flowing agglomerated low-rank coal feedstock.

In a second aspect, the present invention provides a process for gasifying a low-rank coal feedstock to a raw synthesis gas stream comprising carbon monoxide and hydrogen, the process comprising the steps of:

- (A) preparing a low-rank coal feedstock of a specified particle size distribution;
- (B) feeding into a fixed-bed gasifying reactor
- (i) low-rank coal feedstock prepared in step (A), and
- (ii) a gas stream comprising one or both of steam and oxygen;
- (C) reacting low-rank coal feedstock fed into gasifying reactor in step (B), at elevated temperature and pressure, with the gas stream, to generate a raw gas comprising carbon monoxide and hydrogen; and
- (D) removing a stream of the raw gas generated in the gasifying reactor in step (C) as the raw synthesis gas stream, wherein the low-rank coal feedstock comprises a free-flowing agglomerate particulate low-rank coal feedstock, and step (A) comprises the steps of:
  - (a) selecting a specification for the particle distribution of the free-flowing agglomerated particulate low-rank coal feedstock, the specification comprising
    - (i) a target upper end particle size of about 72600 microns of less,
    - (ii) a target lower end particle size of about 6350 microns or greater, and
    - (iii) a target  $dp(50)$  between the target upper end particle size and target lower end particle size;
  - (b) providing a raw particulate low-rank coal feedstock having an initial particle density;
  - (c) grinding the raw particulate low-rank coal feedstock to a ground  $dp(50)$  of from about 2% to about 50% of the target  $dp(50)$ , to generate a ground low-rank coal feedstock;
  - (d) pelletizing the ground low-rank coal feedstock with water and a binder to generate free-flowing agglomerated low-rank coal particles having a pelletized  $dp(50)$  of from about 90% to about 110% of the target  $dp(50)$ , and a particle density of at least about 5% greater than the initial particle density, wherein the binder is selected from the group consisting of a water-soluble binder, a water-dispersible binder and a mixture thereof; and

- (e) removing at least about 90 wt % of (i) particles larger than the upper end particle size, and (ii) particles smaller than the lower end particle size, from the free-flowing agglomerated low-rank coal particles to generate the free-flowing agglomerated low-rank coal feedstock.

The processes in accordance with the present invention are useful, for example, for more efficiently producing higher-value products and by-products from various low-rank coal materials at a reduced capital and operating intensity, and greater overall process efficiency.

These and other embodiments, features and advantages of the present invention will be more readily understood by those of ordinary skill in the art from a reading of the following detailed description.

#### BRIEF DESCRIPTION OF THE DRAWINGS

FIG. 1 is a general diagram of an embodiment of a process for preparing a free-flowing agglomerated particulate low-rank coal feedstock in accordance with the first aspect present invention.

FIG. 2 is a general diagram of an embodiment of a gasification process in accordance with the present invention.

#### DETAILED DESCRIPTION

The present invention relates to processes for preparing feedstocks from low-rank coals that are suitable for use in certain gasification processes, and for converting those feedstocks ultimately into one or more value-added products. Further details are provided below.

In the context of the present description, all publications, patent applications, patents and other references mentioned herein, if not otherwise indicated, are explicitly incorporated by reference herein in their entirety for all purposes as if fully set forth.

Unless otherwise defined, all technical and scientific terms used herein have the same meaning as commonly understood by one of ordinary skill in the art to which this disclosure belongs. In case of conflict, the present specification, including definitions, will control.

Except where expressly noted, trademarks are shown in upper case.

Unless stated otherwise, all percentages, parts, ratios, etc., are by weight.

Unless stated otherwise, pressures expressed in psi units are gauge, and pressures expressed in kPa units are absolute. Pressure differences, however, are expressed as absolute (for example, pressure 1 is 25 psi higher than pressure 2).

When an amount, concentration, or other value or parameter is given as a range, or a list of upper and lower values, this is to be understood as specifically disclosing all ranges formed from any pair of any upper and lower range limits, regardless of whether ranges are separately disclosed. Where a range of numerical values is recited herein, unless otherwise stated, the range is intended to include the endpoints thereof, and all integers and fractions within the range. It is not intended that the scope of the present disclosure be limited to the specific values recited when defining a range.

When the term "about" is used in describing a value or an end-point of a range, the disclosure should be understood to include the specific value or end-point referred to.

As used herein, the terms "comprises," "comprising," "includes," "including," "has," "having" or any other variation thereof, are intended to cover a non-exclusive inclusion. For example, a process, method, article, or apparatus that comprises a list of elements is not necessarily limited to only

those elements but can include other elements not expressly listed or inherent to such process, method, article, or apparatus.

Further, unless expressly stated to the contrary, "or" and "and/or" refers to an inclusive and not to an exclusive. For example, a condition A or B, or A and/or B, is satisfied by any one of the following: A is true (or present) and B is false (or not present), A is false (or not present) and B is true (or present), and both A and B are true (or present).

The use of "a" or "an" to describe the various elements and components herein is merely for convenience and to give a general sense of the disclosure. This description should be read to include one or at least one and the singular also includes the plural unless it is obvious that it is meant otherwise.

The term "substantial", as used herein, unless otherwise defined herein, means that greater than about 90% of the referenced material, preferably greater than about 95% of the referenced material, and more preferably greater than about 97% of the referenced material. If not specified, the percent is on a molar basis when reference is made to a molecule (such as methane, carbon dioxide, carbon monoxide and hydrogen sulfide), and otherwise is on a weight basis (such as for carbon content).

The term "predominant portion", as used herein, unless otherwise defined herein, means that greater than 50% of the referenced material. If not specified, the percent is on a molar basis when reference is made to a molecule (such as hydrogen, methane, carbon dioxide, carbon monoxide and hydrogen sulfide), and otherwise is on a weight basis (such as for carbon content).

The term "depleted" is synonymous with reduced from originally present. For example, removing a substantial portion of a material from a stream would produce a material-depleted stream that is substantially depleted of that material. Conversely, the term "enriched" is synonymous with greater than originally present.

The term "carbonaceous" as used herein is synonymous with hydrocarbon.

The term "carbonaceous material" as used herein is a material containing organic hydrocarbon content. Carbonaceous materials can be classified as biomass or non-biomass materials as defined herein.

The term "biomass" as used herein refers to carbonaceous materials derived from recently (for example, within the past 100 years) living organisms, including plant-based biomass and animal-based biomass. For clarification, biomass does not include fossil-based carbonaceous materials, such as coal. For example, see US2009/0217575A1, US2009/0229182A1 and US2009/0217587A1.

The term "plant-based biomass" as used herein means materials derived from green plants, crops, algae, and trees, such as, but not limited to, sweet sorghum, bagasse, sugar-cane, bamboo, hybrid poplar, hybrid willow, albizia trees, eucalyptus, alfalfa, clover, oil palm, switchgrass, sudangrass, millet, jatropha, and miscanthus (e.g., *Miscanthus x giganteus*). Biomass further include wastes from agricultural cultivation, processing, and/or degradation such as corn cobs and husks, corn stover, straw, nut shells, vegetable oils, canola oil, rapeseed oil, biodiesels, tree bark, wood chips, sawdust, and yard wastes.

The term "animal-based biomass" as used herein means wastes generated from animal cultivation and/or utilization. For example, biomass includes, but is not limited to, wastes from livestock cultivation and processing such as animal manure, guano, poultry litter, animal fats, and municipal solid wastes (e.g., sewage).

The term "non-biomass", as used herein, means those carbonaceous materials which are not encompassed by the term "biomass" as defined herein. For example, non-biomass include, but is not limited to, anthracite, bituminous coal, sub-bituminous coal, lignite, petroleum coke, asphaltenes, liquid petroleum residues or mixtures thereof. For example, see US2009/0166588A1, US2009/0165379A1, US2009/0165380A1, US2009/0165361A1, US2009/0217590A1 and US2009/0217586A1.

10 "Liquid heavy hydrocarbon materials" are viscous liquid or semi-solid materials that are flowable at ambient conditions or can be made flowable at elevated temperature conditions. These materials are typically the residue from the processing of hydrocarbon materials such as crude oil. For example, the first step in the refining of crude oil is normally a distillation to separate the complex mixture of hydrocarbons into fractions of differing volatility. A typical first-step distillation requires heating at atmospheric pressure to vaporize as much of the hydrocarbon content as possible without exceeding an actual temperature of about 650° F. (about 343° C.), since higher temperatures may lead to thermal decomposition. The fraction which is not distilled at atmospheric pressure is commonly referred to as "atmospheric petroleum residue". The fraction may be further distilled under vacuum, such that an actual temperature of up to about 650° F. (about 343° C.) can vaporize even more material. The remaining undistillable liquid is referred to as "vacuum petroleum residue". Both atmospheric petroleum residue and vacuum petroleum residue are considered liquid heavy hydrocarbon materials for the purposes of the present invention.

Non-limiting examples of liquid heavy hydrocarbon materials include vacuum resids; atmospheric resids; heavy and reduced petroleum crude oils; pitch, asphalt and bitumen (naturally occurring as well as resulting from petroleum refining processes); tar sand oil; shale oil; bottoms from catalytic cracking processes; coal liquefaction bottoms; and other hydrocarbon feedstreams containing significant amounts of heavy or viscous materials such as petroleum wax fractions.

40 The term "asphaltenes" as used herein is an aromatic carbonaceous solid at room temperature, and can be derived, for example, from the processing of crude oil and crude oil tar sands. Asphaltenes may also be considered liquid heavy hydrocarbon feedstocks.

45 The liquid heavy hydrocarbon materials may inherently contain minor amounts of solid carbonaceous materials, such as petroleum coke and/or solid asphaltenes, that are generally dispersed within the liquid heavy hydrocarbon matrix, and that remain solid at the elevated temperature conditions utilized as the feed conditions for the present process.

50 The terms "petroleum coke" and "petcoke" as used herein include both (i) the solid thermal decomposition product of high-boiling hydrocarbon fractions obtained in petroleum processing (heavy residues—"resid petcoke"); and (ii) the solid thermal decomposition product of processing tar sands (bituminous sands or oil sands—"tar sands petcoke"). Such carbonization products include, for example, green, calcined, needle and fluidized bed petcoke.

55 Resid petcoke can also be derived from a crude oil, for example, by coking processes used for upgrading heavy-gravity residual crude oil (such as a liquid petroleum residue), which petcoke contains ash as a minor component, typically about 1.0 wt % or less, and more typically about 0.5 wt % or less, based on the weight of the coke. Typically, the ash in such lower-ash cokes predominantly comprises metals such as nickel and vanadium.

60 Tar sands petcoke can be derived from an oil sand, for example, by coking processes used for upgrading oil sand.

Tar sands petcoke contains ash as a minor component, typically in the range of about 2 wt % to about 12 wt %, and more typically in the range of about 4 wt % to about 12 wt %, based on the overall weight of the tar sands petcoke. Typically, the ash in such higher-ash cokes predominantly comprises materials such as silica and/or alumina.

Petroleum coke can comprise at least about 70 wt % carbon, at least about 80 wt % carbon, or at least about 90 wt % carbon, based on the total weight of the petroleum coke. Typically, the petroleum coke comprises less than about 20 wt % inorganic compounds, based on the weight of the petroleum coke.

The term "coal" as used herein means peat, lignite, sub-bituminous coal, bituminous coal, anthracite, or mixtures thereof. In certain embodiments, the coal has a carbon content of less than about 85%, or less than about 80%, or less than about 75%, or less than about 70%, or less than about 65%, or less than about 60%, or less than about 55%, or less than about 50% by weight, based on the total coal weight. In other embodiments, the coal has a carbon content ranging up to about 85%, or up to about 80%, or up to about 75% by weight, based on the total coal weight. Examples of useful coal include, but are not limited to, Illinois #6, Pittsburgh #8, Beulah (ND), Utah Blind Canyon, and Powder River Basin (PRB) coals. Anthracite, bituminous coal, sub-bituminous coal, and lignite coal may contain about 10 wt %, from about 5 to about 7 wt %, from about 4 to about 8 wt %, and from about 9 to about 11 wt %, ash by total weight of the coal on a dry basis, respectively. However, the ash content of any particular coal source will depend on the rank and source of the coal, as is familiar to those skilled in the art. See, for example, "Coal Data: A Reference", Energy Information Administration, Office of Coal, Nuclear, Electric and Alternate Fuels, U.S. Department of Energy, DOE/EIA-0064(93), February 1995.

The ash produced from combustion of a coal typically comprises both a fly ash and a bottom ash, as is familiar to those skilled in the art. The fly ash from a bituminous coal can comprise from about 20 to about 60 wt % silica and from about 5 to about 35 wt % alumina, based on the total weight of the fly ash. The fly ash from a sub-bituminous coal can comprise from about 40 to about 60 wt % silica and from about 20 to about 30 wt % alumina, based on the total weight of the fly ash. The fly ash from a lignite coal can comprise from about 15 to about 45 wt % silica and from about 20 to about 25 wt % alumina, based on the total weight of the fly ash. See, for example, Meyers, et al. "Fly Ash. A Highway Construction Material," Federal Highway Administration, Report No. FHWA-IP-76-16, Washington, D.C., 1976.

The bottom ash from a bituminous coal can comprise from about 40 to about 60 wt % silica and from about 20 to about 30 wt % alumina, based on the total weight of the bottom ash. The bottom ash from a sub-bituminous coal can comprise from about 40 to about 50 wt % silica and from about 15 to about 25 wt % alumina, based on the total weight of the bottom ash. The bottom ash from a lignite coal can comprise from about 30 to about 80 wt % silica and from about 10 to about 20 wt % alumina, based on the total weight of the bottom ash. See, for example, Moulton, Lyle K. "Bottom Ash and Boiler Slag," Proceedings of the Third International Ash Utilization Symposium, U.S. Bureau of Mines, Information Circular No. 8640, Washington, D.C., 1973.

A material such as methane can be biomass or non-biomass under the above definitions depending on its source of origin.

A "non-gaseous" material is substantially a liquid, semi-solid, solid or mixture at ambient conditions. For example,

coal, petcoke, asphaltene and liquid petroleum residue are non-gaseous materials, while methane and natural gas are gaseous materials.

The term "unit" refers to a unit operation. When more than one "unit" is described as being present, those units are operated in a parallel fashion unless otherwise stated. A single "unit", however, may comprise more than one of the units in series, or in parallel, depending on the context. For example, a cyclone unit may comprise an internal cyclone followed in series by an external cyclone. As another example, a pelletizing unit may comprise a first pelletizer to pelletize to a first particle size/particle density, followed in series by a second pelletizer to pelletize to a second particle size/particle density.

The term "free-flowing" particles as used herein means that the particles do not materially agglomerate (for example, do not materially aggregate, cake or clump) due to moisture content, as is well understood by those of ordinary skill in the relevant art. Free-flowing particles need not be "dry" but, desirably, the moisture content of the particles is substantially internally contained so that there is minimal (or no) surface moisture.

The term "a portion of the carbonaceous feedstock" refers to carbon content of unreacted feedstock as well as partially reacted feedstock, as well as other components that may be derived in whole or part from the carbonaceous feedstock (such as carbon monoxide, hydrogen and methane). For example, "a portion of the carbonaceous feedstock" includes carbon content that may be present in by-product char and recycled fines, which char is ultimately derived from the original carbonaceous feedstock.

The term "superheated steam" in the context of the present invention refers to a steam stream that is non-condensing under the conditions utilized, as is commonly understood by persons of ordinary skill in the relevant art.

The term "dry saturated steam" or "dry steam" in the context of the present invention refers to slightly superheated saturated steam that is non-condensing, as is commonly understood by persons of ordinary skill in the relevant art.

The term "HGI" refers to the Hardgrove Grinding Index as measured in accordance with ASTM D409/D409M-11ae1.

The term "dp(50)" refers to the mean particle size of a particle size distribution as measured in accordance with ASTM D4749-87(2007).

The term "particle density" refers to particle density as measured by mercury intrusion porosimetry in accordance with ASTM D4284-12.

When describing particles sizes, the use of "+" means greater than or equal to (e.g., approximate minimum), and the use of "-" means less than or equal to (e.g., approximate maximum).

Although methods and materials similar or equivalent to those described herein can be used in the practice or testing of the present disclosure, suitable methods and materials are described herein. The materials, methods, and examples herein are thus illustrative only and, except as specifically stated, are not intended to be limiting.

#### General Feedstock Preparation Process Information

The present invention in part is directed to various processes for preparing free-flowing agglomerated particulate low-rank coal feedstocks suitable for certain fixed/moving bed gasification processes.

Typically, in fixed/moving bed gasification applications, a generally coarse particle is utilized but is constrained to upper and lower particles limits of about 72600 microns and about 6350 microns, respectively.

The present invention provides in step (a) the setting of the desired final particle size distribution for the end use of the

ultimate free-flowing agglomerated particulate low-rank coal feedstock, including the target dp(50), target upper end particle size (large or “bigs”) and target lower end particle size (small or “fines”). Typically, the target upper end particle size should be at least 200%, or at least three 300%, and in some cases up to 1000%, of the target dp(50); and the target lower end particle size should be no greater than 50%, or no greater than 33%, and in some cases no less than 10%, of the target dp(50).

A person of ordinary skill in the relevant end-use art will readily be able to determine the desired particle size profile for the desired end use. For example, the desired particle size profile for certain gasification processes is detailed below.

In step (b) the raw particulate low-rank coal feedstock is provided.

The term “low-rank coal” is generally understood by those of ordinary skill in the relevant art. Low-rank coals include typical sub-bituminous coals, as well as lignites and peats. Low-ranks coals are generally considered to be “younger” coals than high-rank bituminous coal and anthracite, and tend to have lower particle density, higher porosity, lower fixed carbon content, higher moisture content, higher volatile content and, in many cases, higher inorganic ash content than such high rank coals.

In one embodiment, a raw “low-rank coal” has an inherent (total) moisture content of about 25 wt % or greater (as measured in accordance with ASTM D7582-10e1), a heating value of about 6500 kcal/kg (dry basis) or less (as measured in accordance with ASTM D5865-11a), and a fixed carbon content of about 45 wt % or less (as measured in accordance with ASTM D7582-10e1).

Low-rank coals include typical sub-bituminous coals, as well as lignites and peats. Low-ranks coals are generally considered to be “younger” coals than high-rank bituminous coal and anthracite, and tend to have lower particle density, higher porosity, lower fixed carbon content, higher moisture content, higher volatile content and, in many cases, higher inorganic ash content than such high rank coals.

Typically, the raw low-rank particulate coal feedstocks will have an HGI of about 50 or greater. An embodiment of a low-rank coal for use in the present invention is a coal with an HGI of about 70 or greater, or from about 70 to about 130. In one embodiment, the low-rank coal is a lignite.

Typically, the raw particulate low-rank coal feedstock for use in the present processes will be substantially low-rank coal, or only low-rank coal. Mixtures of two or more different low-rank coals may also be used.

Mixtures of a predominant amount one or more low-rank coals with a minor amount of one or more other non-gaseous carbonaceous feedstocks may also be used as the raw particulate low-rank coal feedstock. Such other non-gaseous feedstocks include, for example, high-rank coals, petroleum coke, liquid petroleum residues, asphaltenes and biomass. In the event of a combination of a low-rank coal with another type of non-gaseous carbonaceous material, to be considered a “raw particulate low-rank coal feedstock” for the purposes of the present invention, the heating value from the low-rank coal component must be the predominant portion of the combination. Expressed another way, the overall heating value of the raw particulate low-rank coal feedstock is greater than 50%, or greater than about 66%, or greater than about 75%, or greater than about 90%, from a low-rank coal source.

As discussed in more detail below, certain other non-gaseous carbonaceous materials may be added at various other steps in the process. For example, such materials may be used to assist in the pelletizing (binding) of the ground low-rank

coal feedstock, such as liquid petroleum residues, asphaltenes and certain biomasses such as chicken manure.

The raw low-rank coal feedstock provided in step (b) is then processed by the grinding to a small particle size, pelletizing to the desired end particle size and then a final sizing, an embodiment of which is depicted in FIG. 1.

In accordance with that embodiment, a raw particulate low-rank coal feedstock (10) is processed in a feedstock preparation unit (100) to generate a ground low-rank coal feedstock (32), which is combined with a binder (35), pelletized and finally sized in a pelletization unit (350), to generate the free-flowing agglomerated low-rank coal feedstock (32+35) in accordance with the present invention.

Feedstock preparation unit (100) utilizes a grinding step, and may utilize other optional operations including but not limited to a washing step to remove certain impurities from the ground low-rank, and a dewatering step to adjust the water content for subsequent pelletization.

In the grinding step, the raw low-rank coal feedstock (10) can be crushed, ground and/or pulverized in a grinding unit (110) according to any methods known in the art, such as impact crushing and wet or dry grinding to yield a raw ground low-rank coal feedstock (21) of a particle size suitable for subsequent pelletization, which is typically to dp(50) of from about 2%, or from about 5%, or from about 10%, up to about 50%, or to about 40%, or to about 33%, or to about 25%, of the ultimate target dp(50).

The particulate raw low-rank coal feedstock (10) as provided to the grinding step may be as taken directly from a mine or may be initially processed, for example, by a coarse crushing to a particle size sufficiently large to be more finely ground in the grinding step.

Unlike typical grinding processes, the ground low-rank coal feedstock (21) is not sized directly after grinding to remove fines, but is used as ground for subsequent pelletization. In other words, in accordance with the present invention, the raw particulate low-rank coal feedstock (10) is completely ground down to a smaller particle size then reconstituted (agglomerated) up to the target particle size.

The present process thus utilizes substantially all (about 90 wt % or greater, or about 95 wt % or greater, or about 98 wt % or greater) of the carbon content of the particulate raw low-rank coal feedstock (10), as opposed to separating out fine or coarse material that would otherwise need to be separately processed (or disposed of) in conventional grinding operations. In other words, the ultimate free-flowing agglomerated particulate low-rank coal feedstock contains about 90 wt % or greater, or about 95 wt % or greater, or about 98 wt % or greater, of the carbon content of the raw particulate low-rank coal feedstock (10), and there is virtually complete usage of the carbon content (heating value) of the particulate raw low-rank coal feedstock (10) brought into the process.

In one embodiment, the particulate raw low-rank coal feedstock (10) is wet ground by adding an aqueous medium (40) into the grinding process. Examples of suitable methods for wet grinding of coal feedstocks are well known to those of ordinary skilled in the relevant art.

In another embodiment, an acid is added in the wet grinding process in order to break down at least a portion of the inorganic ash that may be present in the particulate raw low-rank coal feedstock (10), rendering those inorganic ash components water-soluble so that they can be removed in a subsequent wash stage (as discussed below). This is particularly useful for preparing feedstocks for hydromethanation and other catalytic processes, as certain of the ash components (for example, silica and alumina) may bind the alkali metal catalysts that are typically used for hydromethanation, ren-

## 11

dering those catalysts inactive. Suitable acids include hydrochloric acid, sulfuric acid and nitric acid, and are typically utilized in minor amounts sufficient to lower the pH of the aqueous grinding media to a point where the detrimental ash components will at least partially dissolve.

The raw ground low-rank coal feedstock (21) may then optionally be sent to a washing unit (120) where it is contacted with an aqueous medium (41) to remove various water-soluble contaminants, which are withdrawn as a wastewater stream (42), and generate a washed ground low-rank coal feedstock (22). The washing step is particularly useful for treating coals contaminated with inorganic sodium and inorganic chlorine (for example, with high NaCl content), as both sodium and chlorine are highly detrimental contaminants in gasification and combustion processes, as well as removing ash constituents that may have been rendered water soluble via the optional acid treatment in the grinding stage (as discussed above).

Examples of suitable coal washing processes are well known to those of ordinary skill in the relevant art. One such process involves utilizing one or a series of vacuum belt filters, where the ground coal is transported on a vacuum belt while it is sprayed with an aqueous medium, typically recycle water recovered from the treatment of wastewater streams from the process (for example, wastewater stream (42)). Additives such as surfactants, flocculants and pelletizing aids can also be applied at this stage. For example, surfactants and flocculants can be applied to assist in dewatering in the vacuum belt filters and/or any subsequent dewatering stages.

The resulting washed ground low-rank coal feedstock (22) will typically be in the form of a wet filter cake or concentrated slurry with a water content that will typically require an additional dewatering stage (dewatering unit (130)) to remove a portion of the water content and generate a ground low-rank coal feedstock (32) having a water content suitable for the subsequent pelletization in pelletization unit (350).

Methods and equipment suitable for dewatering wet coal filter cakes and concentrated coal slurries in this dewatering stage are well-known to those of ordinary skill in the relevant art and include, for example, filtration (gravity or vacuum), centrifugation, fluid press and thermal drying (hot air and/or steam) methods and equipment. Hydrophobic organic compounds and solvents having an affinity for the coal particles can be used to promote dewatering.

A wastewater steam (43) generated from the dewatering stage can, for example, be recycled to washing unit (120) and/or sent for wastewater treatment. Any water recovered from treatment of wastewater stream (43) can be recycled for use elsewhere in the process.

The result from feedstock preparation unit (100) is a ground low-rank coal feedstock (32) of an appropriate particle size and moisture content suitable for pelletization and further processing in pelletization unit (350).

Additional fines materials of appropriate particle size from other sources (not depicted) can be added into the feedstock preparation unit (100) at various places, and/or combined with ground low-rank coal feedstock (32). For example, fines materials from other coal and/or pet coke processing operations can be combined with ground low-rank coal feedstock (32) to modify (e.g., further reduce) the water content of ground low-rank coal feedstock (32) and/or increase the carbon content of the same.

Pelletization unit (350) utilizes a pelletizing step and a final sizing step, and may utilize other optional operations including but not limited to a dewatering step to adjust the water content for ultimate use.

## 12

Pelletizing step utilizes a pelletizing unit (140) to agglomerate the ground low-rank coal feedstock (32) in an aqueous environment with the aid of a binder (35) that is water-soluble or water-dispersible. The agglomeration is mechanically performed by any one or combination of pelletizers well known to those of ordinary skill in the relevant art. Examples of such pelletizers include pin mixers, disc pelletizers and drum pelletizers. In one embodiment, the pelletization is a two-stage pelletization performed by a first type of pelletizer followed in series by a second type of pelletizer, for example a pin mixer followed by a disc and/or drum pelletizer, which combination allows better control of ultimate particle size and densification of the agglomerated low-rank coal particles.

Suitable binders are also well-known to those of ordinary skill in the relevant art and include organic and inorganic binders. Organic binders include, for example, various starches, flocculants, natural and synthetic polymers, biomass such as chicken manure, and dispersed/emulsified oil materials such as a dispersed liquid petroleum resid.

Inorganic binders include mineral binders. In one embodiment, the binder material is an alkali metal which is provided as an alkali metal compound, and particularly a potassium compound such as potassium hydroxide and/or potassium carbonate, which is particularly useful in catalytic steam gasification and hydromethanation processes as the alkali metal serves as the catalyst for those reactions (discussed below). In those steam gasification and hydromethanation processes where the alkali metal catalyst is recovered and recycled, the binder can comprise recycled alkali metal compounds along with makeup catalyst as required.

The pelletizing step should result in wet agglomerated low-rank coal particles (23) having a  $dp(50)$  as close to the target  $dp(50)$  as possible, but generally at least in the range of from about 90% to about 110% of the target  $dp(50)$ . Desirably the wet agglomerated low-rank coal particles (23) have a  $dp(50)$  in the range of from about 95% to about 105% of the target  $dp(50)$ .

Depending on the moisture content of the wet agglomerated low-rank coal particles (23), those particles may or may not be free flowing, and/or may not be structurally stable, and/or may have too high a moisture content for the desired end use, and may optionally need to go through an additional dewatering stage in a dewatering unit (150) to generate a dewatered agglomerated low-rank coal feedstock (24). Methods suitable for dewatering the wet agglomerated low-rank coal particles (32) in dewatering stage are well-known to those of ordinary skill in the relevant art and include, for example, filtration (gravity or vacuum), centrifugation, fluid press and thermal drying (hot air and/or steam). In one embodiment, the wet agglomerated low-rank coal particles (23) are thermally dried, desirably with dry or superheated steam.

A wastewater steam (44) generated from the dewatering stage can, for example, be recycled to pelletizing step (140) (along with binder (35)) and/or sent for wastewater treatment. Any water recovered from treatment of wastewater stream (44) can be recycled for use elsewhere in the process.

The pelletization unit (350) includes a final sizing stage in a sizing unit (160), where all or a portion of particles above a target upper end size (large or "bigs") and below a target lower end particle size (fines or "smalls") are removed to result in the free-flowing agglomerated low-rank coal feedstock (32+35). Methods suitable for sizing are generally known to those of ordinary skill in the relevant art, and typically include screening units with appropriately sized

screens. In one embodiment, at least 90 wt %, or at least 95 wt %, of either or both (desirably) of the bigs and smalls are removed in this final sizing stage.

In order to maximize carbon usage and minimize waste, the particles above the target upper end size are desirably recovered as stream (26) and recycled directly back to grinding unit (110), and/or may be ground in a separate grinding unit (170) to generate a ground bigs stream (27) which can be recycled directly back into pelletizing unit (140). Likewise, the particles below the target lower end size are desirably recovered as stream (25) and recycled directly back to pelletizing unit (140).

Other than any thermal drying, all operations in the feedstock preparation stage generally take place under ambient temperature and pressure conditions. In one embodiment, however, the washing stage can take place under elevated temperature conditions (for example, using heated wash water) to promote dissolution of contaminants being removed during the washing process.

The resulting free-flowing agglomerated low-rank coal feedstock (32+35) will advantageously have increased particle density as compared to the initial particle density of the raw particulate low rank feedstock. The resulting particle density should be at least about 5% greater, or at least about 10% greater, than the initial particle density of the raw particulate low rank feedstock.

In one embodiment, the resulting free-flowing agglomerated low-rank coal feedstock has a target  $d_{50}$

#### Gasification Processes

Processes that can utilize the agglomerated low-rank coal feedstocks in accordance with the present invention include certain gasification processes.

As a general concept, gasification processes convert the carbon in a carbonaceous feedstock to a raw synthesis gas stream that will generally contain carbon monoxide and hydrogen, and may also contain various amounts of methane and carbon dioxide depending on the particular gasification process. The raw synthesis gas stream may also contain other components such as unreacted steam, hydrogen sulfide, ammonia and other contaminants again depending on the particular gasification process, as well as any co-reactants and feedstocks utilized.

The raw synthesis gas stream is generated in a gasification reactor. Suitable gasification technologies are generally known to those of ordinary skill in the relevant art, and many applicable technologies are commercially available.

Non-limiting examples of different types of suitable gasification processes are discussed below. These may be used individually or in combination. All synthesis gas generation process will involve a reactor, which is generically depicted as (180) in FIG. 2, where the free-flowing agglomerated particulate low-rank coal feedstock (or a pyrolyzed or devolatilized char thereof) will be reacted to produce the raw synthesis gas stream. General reference can be made to FIG. 2 in the context of the various synthesis gas generating processes described below.

In one embodiment, the gasification process is based on a thermal gasification process, such as a partial oxidation gasification process where oxygen and/or steam is utilized as the oxidant, such as a steam gasification process.

Gasifiers potentially suitable for use in conjunction with the present invention are, in a general sense, known to those of ordinary skill in the relevant art and include, for example, those based on technologies available from Lurgi AG (Sasol) and others.

As applied to coal, and referring to FIG. 2, these processes convert an agglomerated particulate low-rank coal feedstock

(32+35), or a pyrolyzed or devolatilized char thereof, in a reactor (180) such as an oxygen-blown gasifier or steam gasifier, into a syngas (hydrogen plus carbon monoxide) as a raw synthesis gas stream (195) which, depending on the specific process and carbonaceous feedstock, will have differing ratios of hydrogen:carbon monoxide, will generally contain minor amounts of carbon dioxide, and may contain minor amounts of other gaseous components such as methane, steam, tars, hydrogen sulfide, sulfur oxides and nitrogen oxides.

Depending on the particular process, the agglomerated particulate low-rank coal feedstock (32+35) may be fed into reactor (180) at one or more different locations optimized for the particular gasification process, as will be recognized by a person of ordinary skill in the relevant art.

In certain of these processes, air or an oxygen-enriched gas stream (14) is fed into the reactor (180) along with the agglomerated feedstock (32+35). Optionally, steam (12) may also be fed into the reactor (180), as well as other gases such as carbon dioxide, hydrogen, methane and/or nitrogen.

In certain of these processes, steam (12) may be utilized as an oxidant at elevated temperatures in place of all or a part of the air or oxygen-enrich gas stream (14).

The gasification in the reactor (180) will typically occur in a bed (182) of the agglomerated feedstock (32+35) which is contacted by air or oxygen-enrich gas stream (14), steam (12) and/or other gases (like carbon dioxide and/or nitrogen) that may be fed to reactor (180).

In one embodiment (the Lurgi process as mentioned below), gasification takes place in a bed (182), which is referred in the literature as a "fixed" bed or a "moving" bed, which is not fluidized in the sense of a fluidized-bed reactor.

Typically, thermal gasification is a non-catalytic process, so no gasification catalyst needs to be added to the agglomerated feedstock (32+35) or into the reactor (180); however, a catalyst that promotes syngas formation may be utilized.

Typically, carbon conversion is very high in thermal gasification processes, and any residual residues are predominantly inorganic ash with little or no carbon residue. Depending on reaction conditions, thermal gasification may be slagging or non-slagging, where a residue (197) is withdrawn from reactor (180) as a molten (slagging) or solid (non-slagging) ash or char (to the extent there is still appreciable carbon content in the residue). Typically the residue (197) is collected in a section (186) below bed (182) and a grid plate (188) and withdrawn from the bottom of reactor (180), but ash/char may also be withdrawn from the top (184) of reactor (180) along with raw synthesis gas stream (195).

The raw synthesis gas stream (195) is typically withdrawn from the top or upper portion of reactor (180).

The hot gas effluent leaving bed (182) of reactor (180) can pass through a fines remover unit (such as cyclone assembly (190)), incorporated into and/or external of reactor (180), which serves as a disengagement zone. Particles too heavy to be entrained by the gas leaving the reactor (180) can be returned to the reactor (180), for example, to bed (182).

Residual entrained fines are substantially removed by any suitable device such as internal and/or external cyclone separators (190) optionally followed by Venturi scrubbers to generate a fines-depleted raw product stream (193). At least a portion of these fines can be returned to bed (182) via recycle lines (192), (194) and/or (196), particularly to the extent that such fines still contain material carbon content (can be considered char). Alternatively, any fines or ash can be removed via lines (192) and (198).

These thermal gasification processes are typically operated under relatively high temperature and pressure conditions

## 15

and, as indicated above, may run under slagging or non-slagging operating conditions depending on the process and carbonaceous feedstock.

For example, the Lurgi gasifier has a fixed/moving-bed section that operates at a temperature of from about 750° C. to about 1000° C. and a pressure of from about 150 psig (1136 kPa) to about 600 psig (4238 kPa). Suitable particle sizes are relatively coarse, ranging from about +6350 microns to about -76200 microns, with minimal amounts of particles -6350 microns present due to significant processing/fouling issues with smaller particles. The target dp(50) for the Lurgi process is between the target upper and lower particle sizes as discussed above. See, for example, WO2006/082543A1 and US2009/0158658A1.

Reaction and other operating conditions, and equipment and configurations, of the various reactors and technologies are in a general sense known to those of ordinary skill in the relevant art, and are not critical to the present invention in its broadest sense.

## Multi-Train Processes

In the processes of the invention, each process may be performed in one or more processing units. For example, one or more gasification reactors may be supplied with the feedstock from one or more feedstock preparation unit operations. Similarly, the raw product streams generated by one or more reactors may be processed or purified separately or via their combination at various downstream points depending on the particular system configuration.

In certain embodiments, the processes utilize two or more gasification reactors. In such embodiments, the processes may contain divergent processing units (i.e., less than the total number of gasification reactors) prior to the reactors for ultimately providing the carbonaceous feedstock to the plurality of reactors, and/or convergent processing units (i.e., less than the total number of hydromethanation reactors) following the reactors for processing the plurality of raw gas streams generated by the plurality of reactors.

When the systems contain convergent processing units, each of the convergent processing units can be selected to have a capacity to accept greater than a 1/n portion of the total feed stream to the convergent processing units, where n is the number of convergent processing units. Similarly, when the systems contain divergent processing units, each of the divergent processing units can be selected to have a capacity to accept greater than a 1/m portion of the total feed stream supplying the convergent processing units, where m is the number of divergent processing units.

We claim:

1. A process for preparing a free-flowing agglomerated particulate low-rank coal feedstock of a specified particle size distribution, the process comprising the steps of:

- (a) selecting a specification for the particle size distribution of the free-flowing agglomerated particulate low-rank coal feedstock, the specification comprising
  - (i) a target upper end particle size of about 72600 microns of less,
  - (ii) a target lower end particle size of about 6350 microns or greater, and
  - (iii) a target dp(50) between the target upper end particle size and target lower end particle size;
- (b) providing a raw particulate low-rank coal feedstock having an initial particle density;
- (c) grinding the raw particulate low-rank coal feedstock to a ground dp(50) of from about 2% to about 50% of the target dp(50), to generate a ground low-rank coal feedstock;

## 16

(d) pelletizing the ground low-rank coal feedstock with water and a binder to generate free-flowing agglomerated low-rank coal particles having a pelletized dp(50) of from about 90% to about 110% of the target dp(50), and a particle density of at least about 5% greater than the initial particle density, wherein the binder is selected from the group consisting of a water-soluble binder, a water-dispersible binder and a mixture thereof; and

(e) removing about 90 wt % or greater of

- (i) particles larger than the upper end particle size, and
  - (ii) particles smaller than the lower end particle size,
- from the free-flowing agglomerated low-rank coal particles to generate the free-flowing agglomerated low-rank coal feedstock.

2. The process of claim 1, wherein the raw low-rank particulate coal feedstock has a Hardgrove Grinding Index of about 50 or greater.

3. The process of claim 2, wherein the raw low-rank particulate coal feedstock has a Hardgrove Grinding Index of about 70 or greater.

4. The process of claim 3, wherein the raw low-rank particulate coal feedstock has a Hardgrove Grinding Index of from about 70 to about 130.

5. The process of claim 1, wherein the grinding step is a wet grinding step.

6. The process of claim 5, wherein an acid is added in the wet grinding step.

7. The process of claim 1, wherein the process further comprises the step of washing the raw ground low-rank coal feedstock from the grinding step to generate a washed ground low-rank coal feedstock.

8. The process of claim 7, wherein the raw ground low-rank coal feedstock is washed to remove one or both of inorganic sodium and inorganic chlorine.

9. The process of claim 7, wherein the washed ground low-rank coal has a water content, and the process further comprises the step of removing a portion of the water content from the washed ground low-rank coal feedstock to generate the ground low-rank coal feedstock for the pelletizing step.

10. The process of claim 1, wherein the pelletization is a two-stage pelletization performed by a first type of pelletizer followed in series by a second type of pelletizer.

11. The process of claim 1, wherein the particle density of the free-flowing agglomerated low-rank coal particles is at least about 10% greater than the initial particle density.

12. The process of claim 1, wherein the raw particulate low-rank coal feedstock is ground to a ground dp(50) of from about 5% to about 50% of the target dp(50).

13. A process for gasifying a low-rank coal feedstock to a raw synthesis gas stream comprising carbon monoxide and hydrogen, the process comprising the steps of:

- (A) preparing a low-rank coal feedstock of a specified particle size distribution;
- (B) feeding into a fixed-bed gasifying reactor
  - (i) low-rank coal feedstock prepared in step (A), and
  - (ii) a gas stream comprising one or both of steam and oxygen;
- (C) reacting low-rank coal feedstock fed into gasifying reactor in step (B), at elevated temperature and pressure, with the gas stream, to generate a raw gas comprising carbon monoxide and hydrogen; and
- (D) removing a stream of the raw gas generated in the gasifying reactor in step (C) as the raw synthesis gas stream,

wherein step (A) comprises the process as set forth in claim  
**1**.

**14**. The process of claim **13**, wherein step (A) comprises  
the process as set forth in claim **2**.

**15**. The process of claim **14**, wherein step (A) comprises  
the process as set forth in claim **3**.

**16**. The process of claim **15**, wherein step (A) comprises  
the process as set forth in claim **4**.

**17**. The process of claim **15**, wherein step (A) comprises  
the process as set forth in claim **10**.

10

\* \* \* \* \*